

## UNITED STATES PATENT OFFICE

RAYMOND H. LAMBERT, OF ROCHESTER, NEW YORK, ASSIGNOR TO EASTMAN KODAK COMPANY, OF ROCHESTER, NEW YORK, A CORPORATION OF NEW YORK

## PROCESS OF MAKING PHOTOGRAPHIC EMULSIONS

No Drawing. Application filed April 19, 1929. Serial No. 356,607.

This invention relates to a process for the manufacture of photographic emulsion and particularly to a method of washing the emulsion.

5 In the preparation of a photographic light-sensitive emulsion the sensitive substance is usually silver halide. This material is prepared by addition of a soluble silver salt to a soluble halide such as potassium or ammonium halide. In the resulting 10 double decomposition or chemical interchange, one product is the insoluble silver halide. Its stability and sensitivity are largely controlled by the presence of some 15 protective colloid, usually gelatine, during the precipitation of the insoluble silver halide. A stable suspension is thus formed.

There are likewise formed in this reaction 20 soluble inorganic salts that must be removed from the gelatine prior to further treatment and coating it upon photographic plates or film. Many methods for washing out these 25 superfluous salts have been developed since the processes of King and Johnson developed in 1873. In some processes the set 30 gelatine suspension is extruded or cut into fine shreds and then subjected to a washing treatment which may last from 24 to 48 hours. The prior methods have been cumbersome, slow and therefore inefficient.

It is the object of the present invention to 35 provide a method which will overcome many of the disadvantages of the former processes for washing and purifying the gelatine sus- 40 pension.

I have found that if suitable inorganic salts be added to the photographic emulsion, the gelatine may be coagulated therefrom and will settle to the bottom of the container. 45 In settling the gelatine will carry with it substantially all of the silver halide which has been formed in the emulsion, and of course some of the soluble salts which are formed by the interaction of the silver salt with the alkaline halide. The gelatine is in such a form that it may be readily and easily washed free from the soluble salts without the necessity of shredding or extruding that has hitherto been used.

50 The inorganic salts which I have found

suitable for this purpose are the salt-forming elements of the IV group of the Periodic Table, such for example as tin, lead, titanium, cerium, thorium, zirconium, germanium, etc. I have found that the nitrates of 55 these elements are most suitable for my purpose. Other salts, however, that are compatible with the emulsion without in any way affecting the sensitivity of the coating that may result may be used. 60

It is essential that the salt be used in the correct concentration. Too small an amount of the salt results in the coagulation of the gelatine in a slimy relatively non-viscous mass; while too great a concentration of the 65 salt results in a rubbery, tough material from which it is very difficult to wash the soluble salts. Two or three trials will be sufficient to determine the most desirable concentration. In the use of thorium nitrate, for example, 5% by weight of the gelatine present 70 results in a very slowly coagulated gelatine which is of the slimy character; while 20% of thorium nitrate will result in a material which is of the rubbery character. 75

It is best to maintain the temperature for carrying out this coagulation at or below room temperature. For example, at a temperature of from 10° to 20° C. the coagulation or settling of the gelatine requires from 80 two to four hours. Temperatures much above room temperatures should be avoided, as the settling of the gelatine therefrom is considerably retarded in direct proportion to the increase in temperature of the emulsion. 85

When the gelatine has coagulated in the desired form it carries down with it substantially all of the silver halide which has been formed in the gelatine solution or emulsion. 90 The liquid above the coagulated gelatine contains a large proportion of the soluble salt which liquid can be readily decanted. The gelatine material remaining may be very 95 easily washed, as water diffuses very readily throughout the mass. In case any flocculent gelatine remains above the settled gelatine layer, it can be readily separated from the supernatent liquid by simple filtration and 100

can be as readily washed as the main gelatine layer.

The concentration of the gelatine in the solution is not critical, but I have found that 5 gelatine solutions containing as little as from 0.5-1% of gelatine may be readily coagulated by my method. In fact, the gelatine coagulated from such a solution washes more easily and water diffuses more readily through it 10 than it does through a 5% gelatine which has been allowed to set and has been shredded into fine noodles.

The supernatant liquid contains a large 15 proportion of the soluble salts and in a concentration sufficiently great to permit their recovery therefrom to be economically effected. Heretofore there has been little or no recovery of the salts which have been washed from the emulsion due to the cost of concentrating and recrystallizing from the dilute liquors. My procedure makes this 20 operation economically practical due to the high percentage of salts found especially in the decanted layer.

25 After a thorough washing of the gelatine a slight addition of water may be made to the jelly-like mass, and by heating to 60° or 70° C. the material will readily deflocculate. The temperature of deflocculation depends 30 upon the concentration of the coagulating salt used. At this point more gelatine may be added and the emulsion digested as will be well known to those expert in the art.

I will now describe a specific example of 35 carrying out my method of coagulation and washing of the gelatine emulsion, but it will be understood that I shall not be restricted thereby except as indicated in the appended claims. Two liters of a prepared emulsion 40 containing 20 grams of gelatine and the precipitated silver halide in suspension are added with constant stirring to two liters of a solution containing 2 grams of thorium nitrate. The gelatine containing substantially 45 all the silver halide or other suspended insoluble matter settles to the bottom of the container in about 2 to 4 hours at a temperature of 10°-20° C. The mother liquor is decanted and the gelatine layer washed with 50 distilled water until substantially all the soluble salts are removed from it. This subsequent washing is carried out at room temperature or lower. After washing the coagulum is heated to 60° or 70° C. then 30 grams 55 of gelatine in about 200 cc. of water are added while stirring. An emulsion will slowly reform. Water is then added until the final volume of the emulsion is 800-900 cc., when the material is obtained which coats smoothly 60 on a support such as glass or film base.

Such material, when coated on a plate, dries without staining, bumps, or checking, so often found on photographic plates. I have also noted that plates so obtained have more 65 speed, fix more rapidly, and wash more

quickly than ordinary plates. Plates un-subbed, when coated with this material after allowing to stand for some time, showed no stripping or frilling. The tendency of plates to fog during preparation is reduced and on 70 exposure and development an image is obtained which is remarkably clear and with good detail. The presence of these salts likewise acts as a hardener, and the usual hardeners such as alum, formalin, or alcohol need 75 not be used with an emulsion prepared in this way.

Various changes and modifications may be made in the manner of carrying out this process and equivalents of the coagulating salt 80 used without in any way departing from this invention or sacrificing any of the advantages derived therefrom.

Having thus described my invention what I claim as new and desire to secure by Letters 85 Patent is:

1. In the process of preparing gelatino silver halide emulsions from an emulsion containing gelatine and a silver halide, the step which comprises coagulating the gelatine, with occluded silver halide, with a soluble salt of an element of the IV group of the Periodic Table.

2. In the process of preparing gelatino silver halide emulsions from an emulsion containing gelatine and a silver halide, the step which comprises coagulating gelatine, with occluded silver halide, with a soluble salt of thorium.

3. In the process of preparing gelatino silver halide emulsions from an emulsion containing gelatine and a silver halide, the step which comprises coagulating gelatine, with occluded silver halide, with thorium nitrate.

4. In the process of preparing gelatino silver halide emulsions, the step which comprises coagulating a dilute aqueous gelatino-silver halide-containing emulsion with a soluble salt of an element of the IV group of the Periodic Table.

5. In the process of preparing gelatino silver halide emulsions from an emulsion containing gelatine and a silver halide, the step which comprises coagulating the gelatine, with occluded silver halide, with approximately 5 to 20 parts of thorium nitrate for every 100 parts of gelatine present.

6. In the process of preparing gelatino silver halide emulsions from an emulsion containing gelatine and a silver halide, the step which comprises coagulating the gelatine, with occluded silver halide, at a temperature of 10° to 20° C. with approximately 5 to 20 parts of thorium nitrate.

7. In the process of preparing a light-sensitive gelatino silver halide emulsion, the step which comprises adding a soluble salt of an element of the IV group of the Periodic Table to the emulsion thereby coagulating the gelatine and occluding therewith substan- 125

tially all the silver halide contained in the emulsion.

8. In the process of preparing a gelatino silver halide emulsion, the step which comprises adding a soluble salt of an element of the IV group of the Periodic Table to the emulsion, allowing the gelatine, with occluded silver halide, to settle and washing it free from soluble salts.

10. 9. In the process of preparing a gelatino silver halide emulsion, the step which comprises adding a soluble salt of an element of the IV group of the Periodic Table to the emulsion, allowing the gelatine, with occluded silver halide, to settle and decanting the mother liquor.

10. 10. In the process of preparing a gelatino silver halide emulsion, the step which comprises adding a soluble salt of an element of the IV group of the Periodic Table to the emulsion, allowing the gelatine, with occluded silver halide, to settle and decanting the mother liquor, and finally recovering the soluble salts from the mother liquor.

25. 11. In the process of preparing a light-sensitive gelatino silver halide emulsion from an emulsion containing gelatine and a silver halide, the step which comprises adding to the emulsion 5% to 20% (by weight of the 30 gelatine present) of thorium nitrate at a temperature of 10° C. to 20° C., allowing the gelatine, with occluded silver halide, to settle, decanting the mother liquor and washing the coagulated gelatine substantially free from 35 soluble salts.

12. In the process of preparing gelatino silver halide emulsions from an emulsion containing gelatine and a silver halide, the step which comprises coagulating the gelatine, 40 with occluded silver halide, with a soluble salt of an element of the IV group of the Periodic Table, washing the gelatine, adding a small amount of water and the required addition of gelatine, and heating to reform an 45 emulsion.

13. In the process of preparing gelatine emulsions from an emulsion containing gelatine and insoluble suspended matter, the step which comprises coagulating the gelatine, 50 with occluded insoluble suspended matter, with a soluble salt of an element of the IV group of the Periodic Table.

14. In the process of preparing gelatine light sensitive emulsions from an emulsion containing gelatine and insoluble suspended light-sensitive matter, the step which comprises coagulating the gelatine, with occluded light-sensitive matter, with a soluble salt of an element of the IV group of the Pe- 60 riodic Table.

Signed at Rochester, New York, this 16th day of April, 1929.

RAYMOND H. LAMBERT.